

Mar. 27, 1923.

1,449,748.

H. A. GARDNER.

FABRIC FOR AIRSHIPS AND PROCESS OF MAKING SAME.

FILED NOV. 19, 1920.



By

*H.A. Gardner*  
Inventor

*R. H. Blair*

Attorney

Patented Mar. 27, 1923.

1,449,748

# UNITED STATES PATENT OFFICE.

HENRY A. GARDNER, OF WASHINGTON, DISTRICT OF COLUMBIA.

## FABRIC FOR AIRSHIPS AND PROCESS OF MAKING SAME.

Application filed November 19, 1920. Serial No. 425,190.

To all whom it may concern:

Be it known that I, HENRY A. GARDNER, a citizen of the United States, residing at Washington, District of Columbia, have invented new and useful Improvements in Fabrics for Airships and Processes of Making Same, of which the following is a specification.

This invention relates to a water and gas proof fabric and method of manufacturing the same.

An object of the invention is to provide a water-proof, flexible fabric, of low diffusion to prevent the escape of gas.

Another object of the invention is to provide a water and gas proof fabric which is light in weight and relatively inexpensive to manufacture.

A further object of the invention is to provide a novel method of manufacture of the fabric wherein the expense of production is greatly reduced in comparison with all other known methods.

In the manufacture of various objects which are required to be either waterproof or gasproof, such, for instance, as envelopes of non-rigid balloons or gas cells of rigid airships, difficulty has been encountered in securing a relatively inexpensive fabric that is light in weight. The envelope fabric, for instance, used in non-rigid may weigh as high as 16 oz. per square meter, while the goldbeaters skin used on the fabric for gas cells of rigid ships may be prohibitive in cost due to the high cost of the materials used and the extensive labor required in the manufacture of the fabric.

I have heretofore produced a fabric as disclosed in my prior Patent No. 1,381,413 consisting of high strength cotton coated with a tung oil dope that dries largely by polymerization to a flexible film. This fabric might show a low diffusion. In its manufacture, however, I have found that the first coat of oil dope applied causes the fibres of the thread to become raised and rough or liny surfaces to be presented. Singeing and calendering, as well as the application of additional coats of oil dope, are required to lay these threads. Even with these operations it is not always possible to make a perfectly smooth surface. If the fibres are not properly covered, they act as little pores through which hydrogén or other gases and even moisture may ultimately penetrate. I

have, moreover, found that the direct application of an oil product to a fabric such as cotton, for instance, may injure the fabric and cause it to tear very easily. Such fabric also may become brittle or stiff on long exposure.

A suitable method of manufacture will now be described with reference to the accompanying drawing showing a magnified section of the fabric. I select a grade of thread fiber or fabric which is suitable for the purpose intended. When a balloon fabric is desired I prefer either a cotton or a silk cloth of the following construction:

|                           | Cotton.    | Silk.      | 70 |
|---------------------------|------------|------------|----|
| Weight per square yard    | 2.5 oz.    | 2 oz.      |    |
| Width                     | 38 in.     | 38 in.     |    |
| Minimum tensile strength: |            |            | 75 |
| Warp                      | 35 pounds. | 45 pounds. |    |
| Filling                   | 35 "       | 45 "       |    |
| Minimum thread count:     |            |            | 80 |
| Warp                      | 116        |            |    |
| Filling                   | 124        |            |    |

I first fill the fabric indicated at 1, with rubber preferably in solution in benzol or a similar diluent. 10 parts of Pará rubber and 90 parts of benzol will give a satisfactory mixture. If desired, a small amount of sulphur or other vulcanizing agent may be incorporated (usually less than 1%). The filling of the interstices of the first cloth with this mass may be done by brushing, dipping or coating, preferably with a machine. I generally apply from 3 to 8 coats of this composition to each side of the cloth until it is well filled, the pores between the fibers as well as the fibres being covered and rendered into a more or less continuous sheet composition.

The rubber solution is applied in excess to form layers designated at 2, on the outside of the basic material. I then, by any suitable apparatus, dry the fabric by passing the same over heated pipes. The coated cloth will now show a continuous surface without raised threads. The fabric is then subsequently treated with one or more coats of oil dope to form films 3 on the outside of the layers 2. The application of this dope may be made by brushing, dipping or application on a coating machine. The oil

dope used is preferably made on the following formula:—

|   |                 |            |
|---|-----------------|------------|
| 5 | Ester gum       | 125 parts. |
|   | Tung oil        | 250 "      |
|   | Liquid driers   | 20 "       |
|   | Turpentine      | 60 "       |
|   | Mineral spirits | 300 "      |

10 Ester-gum is made from resins such as rosin combined with about 10% glycerine to form a neutral ester.

15 If desired, I may incorporate a pigment such as aluminum powder with the oil dope 4. The oil dries well over the rubberized surface to an extremely smooth film, free from lint or raised threads. It is usually advisable to make two applications of the oil dope. The fabric produced is extremely flexible and soft, and shows a continuously 20 lower diffusion than any heretofore produced with the exception of that in which goldbeaters skin films are present. On weathering, the fabric remains soft and maintains an extremely low diffusion, as low 25 as .2 liters per square meter having been obtained after exposure for several weeks. Moreover, the fabric does not deteriorate in strength and does not become harsh or brittle. Its weight is about 5 ounces per 30 square meter.

35 In some instances I may prefer in manufacturing gas cells or similar objects of this fabric to cut the patterns out of the rubberized cloth, putting the seams together with tape, and then applying the oil dope to the formed object. In any event the result is the same.

40 Without further analysis, the foregoing will so fully reveal the gist of this invention that others can by applying current knowledge readily adapt it for various applications without omitting certain features that, from the standpoint of the prior art, fairly constitute essential characteristics of the

generic or specific aspects of this invention, 45 and therefore such adaptations should and are intended to be comprehended within the meaning and range of equivalency of the following claims.

Having now described my invention what 50 I desire to protect and attain by Letters Patent is:—

1. A gas and waterproof fabric comprising a basic fabric material the interstices of which are impregnated with rubber, and a 55 coating of drying oil upon said basic material.

2. A gas and waterproof fabric comprising a basic fabric material of cotton the interstices of which are impregnated with rubber and a coating of drying oil upon 60 said basic material.

3. A gas and waterproof fabric comprising a basic fabric material the interstices of which are impregnated with rubber, to form 65 a coating on the outside thereof, and a coating of drying oil upon the outside of said film of rubber.

4. The herein described method of manufacturing a gas and waterproof fabric which 70 consists in filling a fabric with rubber solution to constitute a basic material, drying said basic material and coating the outside of the material with dope containing an oil 75 of the class which dries by polymerization.

5. The herein described method of manufacturing a gas and waterproof fabric which consists in filling a fabric with rubber solution containing a vulcanizing agent to constitute a basic material, drying said basic 80 material and coating the outside of the material with a dope containing an oil of the class described which dries by polymerization.

85 Signed at Washington, District of Columbia, this 31st day of August, 1920.

HENRY A. GARDNER.